

## UNITED STATES PATENT OFFICE

CARL AUGUST HAANEN, OF COLOGNE-MULHEIM, AND HANS MËURER, OF COLOGNE, GERMANY, ASSIGNORS TO FELTEN AND GUILLEAUME CARLSWERK ACTIEN GESELLSCHAFT, OF COLOGNE-MULHEIM, GERMANY

## WRAPPING PAPER FOR THE INSULATION OF ELECTRIC CABLES

No Drawing. Application filed July 7, 1925, Serial No. 42,104, and in Germany December 27, 1924.

The insulation of high-tension cables consists of cellulose and impregnating compound. The cellulose is used in the form of unloaded and unsized paper. The cable papers used hitherto, whether smoothed on the calender or not, have a density of from 0.60 to 0.87, the term density signifying the quotient derived from the dry weight per square metre in grams and the calculated 10 volume of a square metre of pulp in cubic metres.

It has now been found that, when using the same quantity of impregnating compound, the resistance to puncture of high-tension cables increases, if by rolling or pressing the paper the volume proportion of cellulose to impregnating compound is raised to a certain favourable point. When the pressure applied exceeds a certain amount, the cellulose fibres are so weakened that the resistance to tearing of the paper is inadmissibly 20 reduced and it can no longer be wrapped on.

The present invention relates to a new method of treating cable papers, which is to 25 be carried out before the papers reach the wrapping machine, the method being based on the recognition of the fact that by it the resistance to puncture of the cable insulation is increased.

According to the invention the resistance to puncture of the cable paper is increased by the density of the paper being increased by 30 rolling under great pressure or by other pressure applying means, but no more than the retention of the necessary tensile strength for wrapping the conductors will allow.

It has been found that the pressures to be applied must be so great that the thickness of the paper is reduced at least by 15% of its 35 original thickness. The pressure of the rollers can be raised to such an extent that the thickness of the paper will be reduced to about 60% and more. Such rolling or pressing pressures correspond to increases of density of from 0.90 to 1.30 and more.

In papers treated in this manner it has been found that in spite of the greater density of the paper the absorbent property is not only retained but is in most cases even 50 increased.

The treatment by rolling under pressure or by other pressure applying means may be carried out after the paper has been impregnated with a suitable impregnating medium, for instance paraffin, cable impregnating 55 compounds or the like. By rolling under pressure or by other pressure applying means the paper is given a smooth surface, which ensures the separate paper layers of the cable insulation lying particularly closely on one 60 another. This latter point is also of great importance in obtaining high resistance to puncture.

## What we claim is:—

A method of increasing the resistance to 65 puncture of wrapping paper for insulating electric cables which consists in subjecting the paper to a pressure which increases the density of the paper above .90 and still retains the necessary tensile strength for wrapping the conductor. 70

In testimony whereof we have signed our names to this specification.

CARL AUGUST HAANEN.  
HANS MËURER.

75

80

85

90

95

100